

No. 813,618.

PATENTED FEB. 27, 1906.

H. S. CHAPMAN & W. M. STONE.  
COATED STRIP AND METHOD OF MAKING THE SAME.  
APPLICATION FILED JULY 10, 1905.

Fig. 1



Fig. 2



Fig. 4



Fig. 5



Fig. 7



Fig. 8



Fig. 10



Fig. 12



Witnesses:

Chas. W. LaRue

W. J. Fanning

Inventors:

Henry S. Chapman

Wilbur M. Stone

by Wilbur M. Stone

Attorney

# UNITED STATES PATENT OFFICE.

HENRY S. CHAPMAN, OF GLENRIDGE, NEW JERSEY, AND WILBUR M. STONE, OF NEW YORK, N. Y., ASSIGNORS TO ARLINGTON COMPANY, A CORPORATION OF NEW JERSEY.

## COATED STRIP AND METHOD OF MAKING THE SAME.

No. 813,618.

Specification of Letters Patent.

Patented Feb. 27, 1906.

Application filed July 10, 1905. Serial No. 269,120.

*To all whom it may concern:*

Be it known that we, HENRY S. CHAPMAN, residing in Glenridge, New Jersey, and WILBUR M. STONE, residing in New York, State 5 of New York, citizens of the United States, have invented certain new and useful Improvements in Coated Strips and Methods of Making the Same, of which the following is a specification.

10 This invention relates to coated strips and to the method of coating the same, and has for its object to furnish a strip of material, particularly such material as is normally liable to deterioration by oxidation or otherwise, with a coating of material impervious to moisture or with a material which will provide a protecting or ornamental cover to the strip.

Our improvement is illustrated in the drawings accompanying this specification, and in which drawings—

Figure 1 is a plan view of a strip embodying our improvements and made in accordance with our improved process. Fig. 2 is a 25 section on line *a a* of Fig. 1. Fig. 3 is a section on line *b b* of Fig. 1. Fig. 4 is a plan view similar to Fig. 1, but showing the coated strip with reinforced edges. Fig. 5 is a section on line *c c* of Fig. 4. Fig. 6 is a section on line *d d* of Fig. 4. Fig. 7 is a plan view of another form of our improvement. Fig. 8 is a section on line *e e* of Fig. 7. Fig. 9 is a section on line *f f* of Fig. 7. Fig. 10 is a vertical section on line *g g* of Fig. 11 of one 35 form of a device by which we carry out a portion of our improved process. Fig. 11 is a plan view of the same. Fig. 12 is a detail plan view of a pair of scraper-jaws for putting on the edge beads of Figs. 4, 5, and 6.

40 When made up with steel strips as a base and a coating of pyroxylin compound, our improved coated strips are especially applicable for use as corset-steels and stiffening-stays for garments and the like, whereby a rustless 45 stiffening-strip is provided and one in which the edges and ends are so rounded as to present no sharp edges or corners to wear or cut through the garments in which they are used. With these ends in view our improvement 50 comprises in one of its forms a strip of suitable material—such as steel, whalebone, bamboo, or other rigid material—having

thereon a seamless incasing coating of celluloid, pyroxylin, rubber, lacquer, or other analogous material which is susceptible of 55 being dissolved for use in carrying out our improved process. Fig. 2 illustrates a cross-section of such a strip in which a base of steel or other suitable material 2 is incased in a 60 seamless coating 3. This coating is applied in liquid form by any suitable means, but preferably continuously to a continuous strip, as hereinafter more fully set forth. In Figs. 10 and 11 we have illustrated one form of an apparatus for applying said coating. This 65 apparatus comprises a tank 20 for holding the solution to be applied to the strip. Said tank is furnished with a hole 21 in the bottom thereof, through which the continuous strip 1 may be passed. Said hole 21 is provided with a gate 22, of leather or some other suitable yielding material, the edges of which will engage the strip and prevent the 70 solution from leaking from the tank. Also when the strip is removed said edges will engage each other to prevent leakage. Extending inwardly through opposite sides of the tank and near the bottom thereof are guides 23 24, and near the top thereof are guides 25 26. These guides have vertical 75 notches in their inner ends, respectively, and which notches engage the strip to be coated and direct it vertically in an unvarying path between the inner ends, respectively, of scraper-jaws 27 28. These jaws are adjustably secured to side walls 29 30 by means of screws 31 32, all respectively. By these 80 means the thickness of the coating applied to the strip may be regulated at will. Guides 23 24 25 26 are adjustable in and out, and 85 wider scraper-jaws may be used, whereby the apparatus may be operated to coat strips of 90 any desired width within its capacity.

In the practice of our improved process we proceed as follows: The tank 20 is first filled 95 with the desired coating solution, preferably to a level somewhat above guides 25 26, so that if the coating fluid is scraped off the edges of the strip by said guides the strip will have opportunity to be recoated before passing between scraper-jaws 27 28. One end of a strip of material 1 which it is desired to coat is then passed upwardly through gate 22 and between the inner ends of guides 23

24 and 25 26, respectively, and thence upwardly between the noses of scraper-jaws 27 28. Said jaws are then adjusted in such proximity to the respective sides of the strip 5 as to scrape off the surplus coating liquid and allow the desired amount to remain thereon. If the coating fluid is sufficiently quick-drying, the continuous coated strip may now be led upward a sufficient distance to give the 10 coating time to dry and may then be coiled or spooled ready for the next step in our process, or if a heavier coating is desired than can be conveniently applied in one operation the strip may be passed through the coating-bath one or more additional times. If the 15 coating liquid is slow in drying, the continuous strips may be cut into handleable lengths—say six to twenty feet—as it passes out from the coating-bath and these lengths hung up 20 or otherwise disposed for drying.

To produce the strip of Figs. 1, 2, and 3, the continuous strip is now cut into suitable lengths, preferably with the ends of each length suitably rounded, as at 4, and then 25 each end is dipped in the coating fluid to furnish a protecting and finishing cap 8 thereon, Figs. 1 and 3.

With some coating fluids—such, for instance, as a solution of celluloid—the tendency 30 thereof in drying is to so shrink on the flat surfaces of the strip as to pull away more or less from the edges thereof, whereby said edges are left insufficiently coated. To remedy this lack or to supply reinforcing edges 35 to the coated strip, even though said strip be equally coated on edges and faces, we proceed as follows: In tank 20 we substitute jaws 37 38 for jaws 27 28. Said jaws 37 38 have their noses cut back on each side at 370 40 380, respectively. Said noses are set in close proximity to the previously coated and dried faces of the strip, all respectively, and the strip fed upwardly therebetween. The coating liquid is thereby scraped off from the 45 middle portions of said coated faces and allowed to remain on the edges of the strip and inreaching a short distance therefrom. Upon drying, a reinforcing-bead 5 5 is thereby formed on each edge, Figs. 4, 5, and 6. The 50 continuous strip may then be cut into suitable lengths and their ends coated, as already described.

Another feature of our invention comprises the applying of an incasing coating to strips 55 previously covered with cloth, paper, or similar materials. By this process we are able to produce a coated strip, Figs. 7, 8, and 9, having a wear-resisting cover of fabric or similar material 6, impregnated and coated with a 60 finishing material 7, waterproof or otherwise, as desired, thereby affording additional strength and beauty to the product. The cloth or paper may be applied by any suitable means to the continuous strip and the

then covered strip be fed through the coating-bath one or more times and with or without a reinforcing-bead formed on the edges thereof, as desired. The strip is then cut up into suitable lengths and the ends capped, as already described in connection with Figs. 1 to 6, inclusive. 65

By "scraping" as herein used is meant a removal by a blade, brush, roller, or any similar means.

Having thus described our invention, we 75 claim—

1. A rigid strip having a seamless incasing coating of semiplastic material and a second coating of similar material on a portion thereof, said second portion forming a reinforcing-bead thereon. 80

2. A rigid strip having a seamless incasing coating of semiplastic material and a second coating of similar material on portions thereof, said second portions forming reinforcing-beads lengthwise thereon. 85

3. A strip having a seamless incasing coating of semiplastic material, a reinforcing-bead on each edge thereof and a reinforcing-cap on each end thereof, said beads and caps 90 being of the same material as the coating.

4. A strip having a seamless incasing coating of semiplastic material, a reinforcing-bead on each edge thereof and a reinforcing-cap on each end thereof, said beads and caps 95 being of the same material as the coating and integral therewith.

5. A strip having a covering of fabric, paper or other material and a seamless incasing coating of semiplastic material thereover and a reinforcing-cap on each end thereof of the same material as the coating. 100

6. A strip having a covering of fabric, paper or other material and a seamless impregnating and incasing coating of semiplastic 105 material thereover and a reinforcing-cap on each end thereof of the same material and integral with the coating.

7. The process of coating strips, comprised in applying a solution of coating material to the strip, drying the solution on the strip, again applying a solution of the coating material to the strip, and scraping off the fluid coating from portions of the strip while allowing it to remain on other portions of the 110 strip. 115

8. The process of coating strips, comprised in passing the strip through a solution of coating material, scraping off the surplus material, drying the solution on the strip, then 120 passing the strip again through the coating material and scraping off the fluid coating from portions of the strip while allowing it to remain on other portions of said strip.

9. The process of coating strips comprised in passing the strip through a solution of coating material, scraping off the surplus material, drying the solution on the strip, then 125

passing the strip again through the coating material, scraping off all of the fluid coating solution from the middle of the faces of the strip while allowing the coating solution to remain on the edges of the strip and on those portions of the faces of the strip contiguous to the edges.

Signed this 23d day of June, 1905, at New York, N. Y., before two subscribing witnesses.

HENRY S. CHAPMAN.  
WILBUR M. STONE.

Witnesses:

JOSEPH R. ENSIGN,  
F. K. BREWSTER.